

## UNITED STATES PATENT OFFICE

2,508,407

PROCESS FOR CLEANING ANIMAL FIBERS  
TO PREPARE SAME FOR SUBSEQUENT  
USE IN TEXTILE OPERATIONS

Manuel Levin, Lowell, Mass.

No Drawing. Application December 27, 1946,  
Serial No. 718,898

7 Claims. (Cl. 8—140)

1

The present invention relates to the treatment of animal fibers and is more particularly concerned with the preparation and cleaning of raw animal fibers for subsequent use in the manufacture of various types of cloths and felts. While the process of the invention is particularly adapted to the preparation and cleaning of raw wool, it is not limited thereto but finds application in the treatment of other animal fibers such as alpaca, mohair, camels' hair and the like.

Naturally, in this old and very well developed art, there have been numerous processes for cleaning raw wool and the like and preparing it for manufacturing operations. Present day methods usually involve a preliminary washing or scouring of the animal fibers in a solution of soap or alkali or with a mixture of both. After scouring, the fibers are either dried or they may be soaked in a solution of sulphuric acid of 1% to 15% concentration by weight. After removing the excess of the acid solution by either pressing or centrifuging, the treated fibers are then dried and baked at a temperature up to 250° F. in order to char the vegetable matter and render it removable by mechanical means. The animal fibers at this stage are usually, although not necessarily, treated in an aqueous alkaline solution to neutralize any sulphuric acid that may be left in the fibers. Then the fibers, if necessary, may be treated with a paint removing solvent to remove any branding paint which may be left in the fibers. The depainting solvent is then washed out with alkaline or neutral soap. The fibers at this point may or may not be soaked in a depitching solution and the depitching solution subsequently washed out, if necessary.

The disadvantages inherent in the foregoing procedural steps are obvious and have been known and appreciated in this art for many years. In the first place, there has always been, and there still remains, the serious problem of disposing of the wash waters and in their disposition there has been created the nuisance of stream pollution and consequent creation of a definite health menace. Secondly, because of the foregoing drastic treatment, the fibers have been necessarily weakened, sometimes to a serious extent, and their ultimate weight is considerably less than it would have been had less drastic methods been available. By far the most harmful of these treatments are those employing strong alkalies and hydrolyzed sulphuric acid. As used herein the term "hydrolyzed" is employed to indicate that the ions of the sulphuric acid solution have become dissociated into electrically charged ions.

Stated differently, the term "hydrolyzed" will be employed to indicate a degree of ionization.

While it is probably unnecessary here so to state, it is obvious that the very number of the 5 prior art treatment steps militates seriously against sound economy of operation.

By the present invention the foregoing and other disadvantages of the prior art are obviated to a great extent. The problem of wash water 10 disposal is obviated entirely, the animal fibers are in no way weakened or reduced in weight and, for reasons to be pointed out hereinafter, the new process represents an optimum in economic operation.

15 The underlying concept of the present invention involves a treatment of animal fibers with a hydrochloric acid solution which is substantially unhydrolyzed or un-ionized. This is accomplished by forming a mixture of a hydrochloric acid 20 solution, of strength to be defined later, with a ketone effective to suppress or inhibit, so to speak, the hydrolysis or ionization of the hydrochloric acid solution. By way of explanation the following may be noted: As is well known, a hydrochloric acid solution is ionized and, when an 25 electric current is passed through such hydrochloric acid solution, the solution will conduct the electric current. Now, if this same hydrochloric acid solution is mixed with a sufficient amount of a ketone, this ionization, and consequent ability of the solution to conduct the current, is inhibited.

Generally, in accordance with the practice of the invention, the following procedural steps are 30 observed: Wool, or other animal fibers, is soaked in a hydrochloric acid solution-ketone mixture, with or without agitation, for from 30 to 60 minutes. Alternatively, the fibers may be soaked in a mixture made up by dissolving dry hydrogen 35 chloride in the ketone. Then the excess solution may or may not be removed either by pressing or centrifuging. At this point the fibers are heated gently to a temperature of 205° F. in order to remove and recover the solvent contained in the fibers. The fibers are then baked at a temperature up to 230° F. for about 10 to 30 minutes to char and render the vegetable matter brittle and removable by mechanical means. Naturally, the higher the concentration of hydrochloric acid 40 employed and the higher the temperature, the shorter the time necessary to destroy the vegetable matter. It should be noted that while the fibers are in the hydrochloric acid solution-ketone mix, the grease, fat and oils contained in 45 the fibers are dissolved through the solvent and on the fibers are dissolved through the sol-

vent action of the ketone and the hydrochloric acid is carried into the vegetable matter much more rapidly than when a water solution is employed. Damage to fibers is reduced to a minimum, since the soaking is accomplished in about one-fourth of the time ordinarily employed with water solution and the acid, because of its un-ionized condition, does not adversely affect the animal fibers. Furthermore, while the grease is being dissolved, practically all the paint and tar present are removed by ketone solvent action.

After baking and removal of the vegetable matter by mechanical means, as by crushing and dusting, the fibers are ready for use in the manufacture of felt or cloth. No neutralization of the hydrochloric acid is necessary because this acid is volatile and has been driven off during the heating steps.

The following may be given as a specific example in the practice of the present invention:

100 lbs. of wool or sheepskins, either green or tanned, are soaked in a solution made up of 36 lbs. of concentrated commercial hydrochloric acid (approximately 35% HCl) and 364 lbs. of methylethyl ketone. Alternatively, the solution may be made up by dissolving 12 lbs. of dry hydrogen chloride in 364 lbs. of methylethyl ketone. The wool or sheepskins are allowed to soak in this mixture, with or without agitation, for 30 minutes. One soaking usually is sufficient, but if a larger amount of dirt is present, the fibers may be rinsed in a second solution prepared as above for about 15 minutes. The wool or skins thus soaked may or may not then be centrifuged to remove the excess solution, although this is not necessary since leaving excess solvent and acid in the wool or skins does no harm. In any event, they are then placed in an oven where gentle heat is first applied (about 205° F.). The temperature is then raised to 225° F. and held for about 30 minutes. At the lower temperature the contained solvent is driven off and recovered, while at the higher temperature, the vegetable matter is charred and rendered removable. After crushing and dusting, the fibers are ready for use without further processing.

Ordinary concentrated hydrochloric acid of commerce contains about 35% dissolved hydrogen chloride gas. In the practice of the invention the ratio of such hydrochloric acid solution to the ketone may vary between 1% of the acid and 99% ketone to 12% of the acid to 88% of the ketone. In keeping with the foregoing explanation with respect to hydrolysis or ionization, it should be borne in mind that the water content of the hydrochloric acid solution-ketone mix must be kept below a point where hydrolysis or ionization would take place. Since up to 12% of 35% hydrochloric acid may be used, and since the latter acid is approximately two-thirds water, it follows that the hydrochloric acid-ketone mixture should not contain over about 8% water.

In the treatment step, methylethyl ketone is preferred, although it is to be understood that other ketones such as acetone, dibutyl ketone, and methyl acetone could be employed.

The ketone employed may be distilled after settling out the dirt, and the clean solvent is then ready for re-use, the grease contained in the solvent being usable as such or it may be refined. At this point it should be mentioned that by prior methods, wool grease (crude lanolin) is recovered to the extent of 25-50% of the total grease removed from the fibers. By the present method, 95-100% of the total grease is

recovered. The dry sediment, which has a high nitrogenous and potash content, may be employed as such as a valuable fertilizer. It is particularly adapted for this purpose because it is absolutely free of sproutable weeds, seeds, and live worm and bug pests in their egg or developed stages.

What is claimed is:

1. In a process for cleaning animal fibers and preparing them for subsequent use in the manufacture of various types of cloths and felts, the step consisting of subjecting said fibers to a mixture of concentrated hydrochloric acid and a ketone effective to inhibit ionization of the hydrochloric acid, said mixture containing not over about 8% water.
2. In a process for cleaning animal fibers and preparing them for subsequent use in the manufacture of various types of cloths and felts, the step consisting of subjecting said fibers to a mixture of concentrated hydrochloric acid and a ketone effective to inhibit ionization of the hydrochloric acid, the ratio of acid to ketone being between 1% acid to 99% ketone and 12% acid to 88% ketone, said mixture containing not over about 8% water.
3. In a process for cleaning animal fibers and preparing them for subsequent use in the manufacture of various types of cloths and felts, the step consisting of subjecting said fibers to a mixture of concentrated hydrochloric acid and methylethyl ketone, said mixture containing not over about 8% water.
4. In a process for cleaning animal fibers and preparing them for subsequent use in the manufacture of various types of cloths and felts, the step consisting of subjecting said fibers to a mixture of concentrated hydrochloric acid and acetone, said mixture containing not over about 8% water.
5. In a process for cleaning animal fibers and preparing them for subsequent use in the manufacture of various types of cloths and felts, the step consisting of subjecting said fibers to a mixture of concentrated hydrochloric acid and dibutyl ketone, said mixture containing not over about 8% water.
6. In a process for cleaning animal fibers and preparing them for subsequent use in the manufacture of various types of cloths and felts, the steps consisting of subjecting said fibers to a mixture of concentrated hydrochloric acid, and a ketone effective to inhibit ionization of the hydrochloric acid, removing excess solution-mixture, heating the fibers to drive off the ketone, recovering the ketone, and further heating to char the vegetable matter contained in and on the fibers, said mixture containing not over about 8% water.
7. In a process for cleaning animal fibers and preparing them for subsequent use in the manufacture of various types of cloths and felts, the steps consisting of subjecting said fibers to a solution of dry hydrogen chloride in a ketone effective to inhibit ionization of the hydrochloric acid, removing excess mixture, heating the fibers to drive off the ketone, recovering the ketone, and further heating to char the vegetable matter contained in and on the fibers, said solution containing not over about 8% water.

MANUEL LEVIN.

(References on following page)

## REFERENCES CITED

The following references are of record in the file of this patent:

## UNITED STATES PATENTS

| Number    | Name            | Date          |    |
|-----------|-----------------|---------------|----|
| 549,532   | Rice et al.     | Nov. 12, 1895 |    |
| 1,615,783 | Bergmann et al. | Jan. 25, 1927 |    |
| 1,686,837 | Pott            | Oct. 9, 1928  | 10 |
| 2,155,161 | Fabian et al.   | Apr. 18, 1939 |    |
| 2,393,712 | Seymour et al.  | Jan. 29, 1946 |    |

## FOREIGN PATENTS

| Number  | Country       | Date          |
|---------|---------------|---------------|
| 307,944 | Great Britain | Mar. 11, 1929 |

## OTHER REFERENCES

Clafin, "Phys. Chem. of the Carbonizing Process," Amer. Dyest. Rep. XXI No. 20 (Sept. 26, 1932), pages 575-577.